

June 6, 1939.

F. R. HENSEL ET AL

2,161,467

ALLOY

Filed June 15, 1937

2 Sheets-Sheet 1



June 6, 1939.

F. R. HENSEL ET AL

2,161,467

ALLOY

Filed June 15, 1937

2 Sheets-Sheet 2



*Fig. 2a*

COLD WORK AFTER AGEING

QUENCHED FROM 950°C  
AGED 32 HOURS AT 450°C



*Fig. 3*

HARDNESS & ELECT.  
CONDUCTIVITY VS. AGEING  
TIME

QUENCHED FROM 950°C  
AGED AT 450°C

○ - CONDUCTIVITY  
△ - HARDNESS



*Fig. 3a*

COLD WORK AFTER AGEING

QUENCHED FROM 950°C  
AGED 32 HOURS AT 450°C

INVENTORS  
FRANZ R. HENSEL  
BY EARL I. LARSEN

*John F. O'Brien*  
ATTORNEY

## UNITED STATES PATENT OFFICE

2,161,467

## ALLOY

Franz R. Hensel and Earl I. Larsen, Indianapolis,  
Ind., assignors to P. R. Mallory & Co., Inc.,  
Indianapolis, Ind., a corporation of Delaware

Application June 15, 1937, Serial No. 148,283

## 2 Claims. (Cl. 219—4)

This invention relates to alloys, and more particularly to copper alloys of improved characteristics. The object of the invention is to produce an improved copper base alloy.

5 Another object is to produce a copper zinc alloy of comparatively low zinc content, which can be hardened by means of the addition of a small percentage of zirconium to a higher degree than has heretofore been possible.

10 Another object is to produce a copper alloy which has an excellent combination of hardness, electrical conductivity and resistance to annealing.

15 Further objects are to produce alloys which are readily handled in the mill having a high degree of fluidity in the liquid state and producing sound, clean billets, which are ideally suited for further manufacturing, showing no tendencies of season or fire cracking.

20 Specific objects are the provision of improved copper-zirconium-zinc alloys especially suitable for fabrication into welding electrodes, high strength sand castings for use with cylinder heads, pistons and other parts of internal combustion engines, commutator segments, trolley wires, collector rings, switch plates, bolts, nuts and in general for all uses where high strength and/or high conductivity are required at elevated temperatures.

25 Other objects of the invention will be apparent from the following description taken in connection with the appended claims.

The present invention comprises a combination of elements, methods of manufacture and the product thereof brought out and exemplified 35 in the disclosure hereinafter set forth, the scope of the invention being indicated in the appended claims.

In the drawing:

Figures 1, 2 and 3 are graphs showing curves 40 illustrating the improvement during age hardening in the hardness and electrical conductivity of alloys containing various percentages of zirconium and zinc as follows:

## 45 Figure 1—

|           | Per cent |
|-----------|----------|
| Zirconium | 0.48     |
| Zinc      | 0.62     |
| Copper    | Balance  |

## 50 Figure 2—

|           | 0.85    |
|-----------|---------|
| Zirconium | 0.85    |
| Zinc      | 0.55    |
| Copper    | Balance |

## 55 Figure 3—

|           | 0.97    |
|-----------|---------|
| Zirconium | 0.97    |
| Zinc      | 1.79    |
| Copper    | Balance |

Figures 1a, 2a and 3a are graphs showing the 60 effects of cold working of the alloys referred to

in Figures 1, 2 and 3, respectively, after age hardening.

While a preferred embodiment of the invention is described herein, it is contemplated that considerable variation may be made in the method of procedure and the combination of elements, without departing from the spirit of the invention.

Alloys of copper and zinc in various proportions have been made and used commercially 10 for many years. These alloys in the cast form are quite soft and can only be hardened to a very limited extent by cold working. As a matter of fact, a zinc alloy containing 5% zinc, known generally as gilding metal, can not be work hardened appreciably harder than pure copper. Furthermore the increased hardness can only be retained at fairly low temperatures. If these alloys are heated very substantially, the hardness is lost and can only be regained by further cold 20 working.

Copper zirconium alloys on the other hand, while having many desirable properties, offer certain difficulties in casting and working, which we have found are overcome by the addition of 25 suitable percentages of zinc.

According to the preferred method of carrying out the present invention, an alloy is made containing copper, zinc and zirconium in substantially the following proportions:

|           | Per cent  |
|-----------|-----------|
| Zinc      | 0.1 to 10 |
| Zirconium | 0.1 to 5  |
| Copper    | Balance   |

It is possible likewise to improve the characteristics of other copper zinc alloys containing small percentages of additional ingredients by the addition of zirconium. Thus copper zinc alloys containing small proportions of silver, cadmium, calcium, lithium, silicon, aluminum, magnesium, 40 titanium or beryllium can be improved by the addition of zirconium in substantially the proportions indicated above.

The addition of zirconium to the above alloys renders them susceptible to age hardening. 45

The alloy can be made according to standard alloying methods. A preferred method of alloying is to prepare a "hardener alloy" containing 1-50% zirconium and then introduce a predetermined amount of this alloy into a copper zinc 50 alloy of the desired composition.

After the alloy has been prepared according to the standard alloying methods the heat treatment may be carried out as follows:

The alloy in the form of a billet or any other 55 form, such as a sand casting or a rolled, forged or extruded bar, is raised in temperature to above 700° C. and preferably to a temperature in the order of 700-1000° C. The alloy is then quenched from this high temperature and subsequently 60

aged at a temperature below 700° C. and preferably in the range of between 400-600° C. This heat treatment results in a considerable improvement in hardness of the alloy, as can be seen 5 from the figures.

We have also found that we can quench the 10 alloy in any desirable form and then apply a certain amount of cold working. Alloys of the nature described have been found to be particularly suitable for cold working in the quenched condition. While the alloy, after quenching, will 15 show a minus Rockwell B hardness, cold working after quenching might raise this hardness to a Rockwell B number in the neighborhood of 60-70. After this cold working operation, the 20 material is aged in the range between 350-600° C. Due to the cold working after quenching, a lower temperature or a shorter time may be employed for the aging operation, thus bringing about a material reduction in cost of manufacture, when compared with the usual long drawn out aging operations.

After aging, the material can be still further hardened by applying cold work up to 75% reduction in area. The above described treatments consisting in heat treatments and mechanical workings, have a remarkable effect on the electrical conductivity, as shown in Figures 1, 2 and 3. Values of electrical conductivity 25 ranging from 65-85% can be readily obtained within the percentage ranges given.

This alloy is therefore well suited for use at 30 comparatively high temperatures since hardness and electrical conductivity are maintained for 35 indefinite periods at the aging temperatures indicated.

It was found that the alloys can be cold worked 35 after complete aging as much as 80-90% without losing more than 1-2% in electrical conductivity. 40 This makes the alloy particularly suitable for severe drawing operations, and for use in wire

form where high strength and high conductivity is required, such as for instance, trolley wire. The alloys prepared as indicated are well suited for a large number of purposes. They may be used in the form of sand castings, chill or permanent mold castings, forgings, rolled, extruded or drawn stock, for such applications as commutator segments, collector rings, switch plates, bolts, nuts, and for all parts where special electrical requirements or high heat conductivity 10 and resistance to high temperatures are needed. 5

The alloys are especially adapted for fabrication into resistance welding electrodes, such as spot welding tips, welding wheels, flash welding dies, etc.

Since the addition of zinc makes the alloy quite fluid, it is very well suited for high strength sand castings, such as cylinder heads, pistons and other parts of internal combustion engines, such as automobile engines, where high heat 20 conductivity is needed. 15

While the present invention, as to its objects and advantages, has been described herein as carried out in specified embodiments thereof, it is not desired to be limited thereby, but it is intended to cover the invention broadly within the spirit and scope of the appended claims. 25

What is claimed is:

1. A pressure exerting electrode composed of about 0.1-10% zinc, 0.1-5% zirconium, and the remainder copper. 30

2. A pressure exerting electrode composed of about 0.1-10% zinc, 0.1-5% zirconium, and the remainder substantially all copper, characterized by a combination of high hardness and high 35, electrical conductivity, and further characterized by the ability to maintain its hardness and high conductivity at temperatures in the order of 450° C.

FRANZ R. HENSEL. 40  
EARL I. LARSEN.